

# United States Patent [19]

Hotomi et al.

[11] Patent Number: 4,939,054

[45] Date of Patent: \* Jul. 3, 1990

[54] PHOTORESISTIVE MEMBER COMPOSED  
OF AMORPHOUS CARBON CHARGE  
TRANSPORTING LAYER AND CHARGE  
GENERATING LAYER

[75] Inventors: Hideo Hotomi, Saita; Izumi Osawa,  
Ikeda; Mitsutoshi Nakamura, Osaka;  
Shuji Iino, Hirakata, all of Japan

[73] Assignee: Minolta Camera Kabushiki Kaisha,  
Osaka, Japan

[\*] Notice: The portion of the term of this patent  
subsequent to May 3, 2005 has been  
disclaimed.

[21] Appl. No.: 382,015

[22] Filed: Jul. 18, 1989

## Related U.S. Application Data

[63] Continuation of Ser. No. 34,920, Apr. 6, 1987, abandoned.

## Foreign Application Priority Data

Apr. 9, 1986 [JP] Japan 61-83128  
Apr. 9, 1986 [JP] Japan 61-83129  
Apr. 9, 1986 [JP] Japan 61-83132

[51] Int. Cl.<sup>5</sup> G03G 5/14

[52] U.S. Cl. 430/58

[58] Field of Search 430/58, 60, 66

## References Cited

### U.S. PATENT DOCUMENTS

3,573,906 4/1971 Goffe 430/58  
3,956,525 5/1976 Yasuba 427/41  
4,366,208 12/1982 Akai et al. 204/192  
4,376,688 3/1983 Caesar et al. 204/192  
4,416,755 11/1983 Caesar et al. 204/192  
4,495,262 1/1985 Matsuzaki et al. 430/58  
4,510,224 4/1985 Yamazaki et al. 430/57  
4,518,670 5/1985 Matsuzaki et al. 430/58  
4,544,617 10/1985 Mort et al. 430/58  
4,557,987 12/1985 Shirai et al. 430/58  
4,559,289 12/1985 Sunagawa et al. 430/66  
4,579,801 4/1986 Yashiki 430/60

(List continued on next page.)

## FOREIGN PATENT DOCUMENTS

56-62254 5/1981 Japan .  
60-63541 of 1985 Japan .  
60-67955 4/1985 Japan ..... 430/66  
1174171 12/1989 United Kingdom .

## OTHER PUBLICATIONS

"Photosensitive Materials for Electron Photography-OPC vs. Inorganics", *Nikkei New Materials*, Dec. 15, 1986.

(List continued on next page.)

Primary Examiner—Roland E. Martin

Attorney, Agent, or Firm—Burns, Doane, Swecker & Mathis

[57]

## ABSTRACT

The practice of this invention provides a photosensitive member which comprises a charge transporting layer and a charge generating layer, said charge transporting layer comprising amorphous carbon containing hydrogen, said amorphous carbon comprising hydrogen bonded carbon N<sub>1</sub>, and carbon N<sub>2</sub> free from linking with hydrogen, the ratio of the amount of N<sub>1</sub> to that of N<sub>2</sub> being 1:0.1 to 1:1, and said hydrogen being contained in an amount of 20 to 67 atomic %; or said amorphous carbon comprising unsaturated carbon N<sub>3</sub> linked with hydrogen and saturated carbon N<sub>4</sub> linked with hydrogen, the ratio of the amount of N<sub>3</sub> to that of N<sub>4</sub> being 1:1 to 1:16, said hydrogen being contained in an amount of 20 to 67 atomic %; or said amorphous carbon comprising unsaturated compound N<sub>5</sub> free from linking with hydrogen and saturated carbon N<sub>6</sub> free from linking with hydrogen, the ratio of the amount of N<sub>5</sub> to that of N<sub>6</sub> being 1:20 to 1:0.5, said hydrogen being contained in an amount of 20 to 67 atomic %.

The photosensitive member obtained thereby is excellent in charge-transporting property and chargeability and, moreover, exhibits advantages in corona resistance and resistances to acids, moisture and heat and also in physical properties such as stiffness.

7 Claims, 4 Drawing Sheets



## U.S. PATENT DOCUMENTS

|           |        |                 |          |
|-----------|--------|-----------------|----------|
| 4,634,648 | 1/1987 | Jansen et al.   | 430/84   |
| 4,675,265 | 6/1987 | Kazama et al.   | 430/66 X |
| 4,741,982 | 5/1988 | Iino et al.     | 430/58   |
| 4,755,444 | 7/1988 | Karakida et al. | 430/66   |

## OTHER PUBLICATIONS

*A Review of Recent Advances in Plasma Polymerization*,  
by Shen and Bell, Department of Chemical Engineering,  
U. of California, Berkley, CA, 94720.

"Properties of Diamond-Like Carbon Films", *Thin Solid Films*, vol. 119, pp. 121-126, 1984.

"Electronic Properties of Substitutionally Doped Amorphous Si and Ge", *Philosophical Magazine*, vol. 33, No. 6, pp. 935-949, 1976.

"A C-NMR Investigation of Plasma Polymerized Ethane, Ethylene, and Acetylene", by A. Dilks, S. Kaplan, and A. Vanlaeken, Xerox Webster Research Center, Xerox Square, W-114, Rochester, N.Y. 14644.

Fig. 1



Fig. 2



Fig. 3



Fig. 4



Fig. 5



Fig. 6



Fig. 7



Fig. 8



Fig. 9



Fig. 10



Fig. 11



Fig. 12





*Fig. 14*



Fig. 15



**PHOTOSENSITIVE MEMBER COMPOSED OF  
AMORPHOUS CARBON CHARGE  
TRANSPORTING LAYER AND CHARGE  
GENERATING LAYER**

This application is a continuation of application Ser. No. 034,920, filed Apr. 6, 1987 now abandoned.

**BACKGROUND OF THE INVENTION**

This invention relates to a photosensitive member and, more particularly, to a photosensitive member in electrophotography.

Amorphous silicon (hereinafter abbreviated to "a-Si"), made by the plasma chemical vapor deposition process (hereinafter called "plasma CVD process"), has in recent years been finding application as a photosensitive material, especially in electrophotography.

The photosensitive material a-Si has various splendid properties. However, its use raises a problem that, because of a large specific inductive capacity epsilon of approximately 12, a-Si essentially needs to form a film with a minimum thickness of approximately 25 microns in order for the photosensitive member to have a sufficient surface potential.

The production of a-Si photosensitive members by the plasma CVD process is a time-consuming operation with the a-Si film formed at a slow rate of deposition, and, moreover, the more difficult it becomes to obtain a-Si films of uniform quality, the longer it takes for the films to be formed. Consequently, there is a high probability that an a-Si photosensitive member causes defects in images when used, such as white spot noise, besides other defects including an increase in cost of the raw material.

In any attempt for improvement that has been made concerning the above-mentioned defects, it was essentially undesirable to make the film thickness smaller than the minimum mentioned above.

Furthermore, the a-Si photosensitive material exhibits defects in adhesivity to the substrate, in corona resistance and resistance to environment and also chemicals.

As an answer to the problems described above, it has been proposed to provide an a-Si photosensitive layer with an overcoating layer or an undercoating layer of an organic plasma-polymerized film: examples describing the overcoating were announced in Japanese Patent KOKAI Nos. 61761/1985, 214859/1984, 46130/1976, U.S. Pat. No. 3,956,525, etc. and those describing the undercoating in Japanese Patent KOKAI Nos. 63541/1985, 136742/1984, 38753/1984, 28161/1984, etc.

As other prior art disclosing an application of plasma polymerization there are known Japanese Patent KOKAI Nos. 148326/84, 60447/81, and 120527/78.

It is known that an organic plasma-polymerized film can be made from any of gaseous organic compounds, such as ethylene gas, benzene and aromatic silane, (one reference in this respect is the Journal of Applied Polymer Science 1973, 17 (885-892) contributed by A. T. Bell, M. Shen et al.), but any such organic plasma-polymerized film produced by a conventional method has been in use only where its insulation property is required to be good. Films of this kind have been regarded as insulators having electrical resistance of approximately  $10^{16}$  ohm cm, such as an ordinary polyethylene film, or at the least as materials practically similar to an insulator in the application.

The Japanese Patent KOKAI No. 61761/1985 made public a photosensitive member coated with a surface protective layer which is a carbon insulation film resembling diamond with a film thickness of 500 angstrom-2 microns. This thin carbon film is designed to improve a-Si photosensitive members with respect to their resistance to corona discharge and mechanical strength. The polymer film is very thin and an electric charge passes within the film by a tunnel effect, the film itself not

10 needing an ability to transport an electric charge. The publication lacked a description of a carrier-transporting property of the organic plasma-polymerized film and failed to provide a solution to the essential problems of a-Si in the foregoing description.

15 The Japanese Patent KOKAI No. 214859/1984 made public the use of an overcoating layer of an organic transparent film with a thickness of approximately 5 microns, which can be made from an organic hydrocarbon monomer, such as ethylene and acetylene, by a

20 technique of plasma polymerization. The layer described therein was designed to improve a-Si photosensitive members with respect to separation of the film from the substrate, durability, pinholes, and production efficiency. The publication lacked a description relating

25 to a carrier-transporting property of the organic plasma-polymerized film and the topic matter failed to provide a solution to the essential problems of set forth in the foregoing description.

The Japanese Patent KOKAI No. 46130/1976 made 30 public a photosensitive member utilizing n-vinylcarbazole, wherein an organic plasma-polymerized film with thickness of 3 microns-0.001 microns was formed at the surface by a technique of glow discharge. The purpose of this technique was to make bipolar charging

35 applicable to a photosensitive member of poly-n-vinylcarbazole, to which otherwise only positive charging had been applicable. The plasma-polymerized film is produced in a very thin layer of 0.001 microns-3 microns and used by way of overcoating. The polymer layer is very thin, and it is not considered necessary for

40 it to have the ability to transport an electric charge. The publication lacked a description relating to the carrier transporting property of the polymer layer and the topic matter failed to provide a solution to the essential problems of a-Si in the foregoing description.

The United States Patent Publication U.S. Pat. No. 3,956,525 made public a technique whereby on a substrate a layer of a sensitizer is laid and thereupon a layer of an organic photoconductive electric insulator is superimposed and the laminate is overlaid by a polymer film 0.1 micron-1 micron thick formed by a technique of glow discharge. This film is designed to protect the surface so as to make the photosensitive members resistant to wet developing and therefore used by way of overcoating. The polymer film is very thin and does not need an ability to transport an electric charge. The publication lacked a description relating to the carrier transporting property of the polymer film and the topic matter failed to provide a solution to the essential problems of a-Si in the foregoing description.

45 The Japanese Patent KOKAI No. 63541/1985 made public a photosensitive member wherein an a-Si layer is undercoated by an organic plasma-polymerized film resembling diamond with a thickness of 200 angstrom to 2 microns. The organic plasma-polymerized film is designed to improve the adhesivity of the a-Si layer to the substrate. The polymer film can be made very thin and an electric charge passes within the film by a tunnel

effect, the film itself not needing an ability to transport an electric charge. The publication lacked a description relating to the carrier transporting property of the organic plasma-polymerized film and the topic matter failed to provide a solution to the essential problems of a-Si in the foregoing description.

The Japanese Patent KOKAI No. 136742/1984 described a semiconductor device wherein on a substrate an organic plasma-polymerized layer with thickness of approximately 5 microns was formed and thereon a silicon layer was superimposed. Said organic plasma-polymerized layer was designed to prevent the aluminum, the material forming the substrate, from diffusing into the a-Si, but the publication lacked description relating to the method of its fabrication, its quality, etc. The publication also lacked a description relating to the carrier transporting property of the organic plasma-polymerized layer and the topic matter failed to provide a solution to the essential problems of a-Si in the foregoing description.

The Japanese Patent KOKAI No. 28161/1984 made public a photosensitive member wherein on a substrate an a-Si film is laid and thereupon an organic plasma-polymerized film is superimposed. The organic plasma-polymerized film is used as an undercoat, the insulation property thereby being utilized, and also has the functions of blocking, improving the adhesivity, or preventing the separation of the photosensitive coat.

The polymer layer may be very thin (e.g. less than 5 micron meter, preferably less than 1 micron meter). Such a thin layer does not cause any problems such as increase of surface potential (residual potential) even if it has insufficient charge transportability, because the residual potential is controlled at a lower level by the increase of the electric potential at an undercoat layer by repeated use and the enlargement of pass of carrier thereby (tunnel effect). Therefore, this polymer layer can be used as an undercoat layer but cannot be used as a carrier transporting layer.

Further, this prior art does not refer to carrier transportability due to an a-C layer, and it does not dissolve the essential problem caused by an a-Si as aforementioned.

The Japanese Patent KOKAI No. 38753/1984 made public a technique whereby an organic plasma polymerized thin film with a thickness of 10-100 angstrom is formed from a mixed gas composed of oxygen, nitrogen and a hydrocarbon, by a technique of plasma polymerization and thereupon an a-Si layer is formed. Said organic plasma-polymerized film is not deteriorated by heat in comparison with other organic polymers and used as an undercoat utilizing the insulation property of the polymer and also has the functions of blocking or preventing the separation of the photosensitive coat. The polymer film can be made very thin and an electric charge passes within the film by a tunnel effect, the film itself not needing an ability to transport an electric charge. The publication lacked a description relating to the carrier transporting property of the organic plasma-polymerized film and the topic matter failed to provide a solution to the essential problems of a-Si in the foregoing description.

Japanese Patent KOKAI No. 148326/81 discloses a production of a plasma-CVD thin layer comprising a pre-decomposition of gas and a pre-polymerization. However, Si compounds are only exemplified in the Examples.

The Japanese Patent KOKAI No. 60447/1981 made public a method of forming an organic photoconductive layer by plasma polymerization. The publication lacked description relating to the applicability of the invention to electrophotography. The description in the publication dealt with said layer as a charge generating layer or a photoconductive layer and the invention described thereby differs from the present invention. The topic matter failed to provide a solution to the essential problems of a-Si in the foregoing description.

Japanese Patent KOKAI No. 120527/78 discloses a production of a posi-type radial sensitive layer by a plasma polymerization of hydrocarbon and halogenized hydrogen. This is a production of posi-type resist material by cross-linkage using an electron-ray, X-ray,  $\lambda$ -ray or alpha-ray, which is not applied to an electrophot-sensitive member.

As aforementioned in the photosensitive a-C layers have been used as an undercoat layer or overcoat layer, which does not need a carrier transportability, and is used under the recognition that the organic polymer film is an insulator. Therefore, the film is only used as a thin film of at most 5 micron meter or so, and a carrier passes through the film due to a tunnel effect. Where the tunnel effect cannot be expected, the film can be used only at such a thin thickness that a residual potential is practically negligible.

The inventors of the invention found that organic polymerized layer recognized as an insulator have variable electric resistance, in proportion to the ratio of the amount of carbon with certain specific bonding types (such as, carbon-carbon double bonds, or quaternary carbon), and that they begin to have charge transporting properties at a certain ratio thereof.

#### SUMMARY OF THE INVENTION

The primary object of this invention is to provide a photosensitive member which is free from the above-mentioned defects, good in electric charge-transporting properties and electrical chargeability, and ensures formation of satisfactory images.

Another object of this invention is to provide a photosensitive member which is capable of assuming a sufficient surface potential even when the thickness of the layer is small.

Another object of this invention is to provide a photosensitive member which can be fabricated at low cost and in a short time.

Another object of this invention is to provide a photosensitive member which has an amorphous carbon layer which is good in resistances to corona discharge, acids, humidity and heat, and in stiffness.

These objects and other related objects can be accomplished by providing a photosensitive member which comprises an electrically conductive substrate, a charge generating layer, and a charge transporting layer comprising amorphous carbon containing hydrogen, said amorphous carbon comprising hydrogen bonded carbon  $N_1$ , and carbon  $N_2$  free from linking with hydrogen, the ratio of the amount of  $N_1$  to that of  $N_2$  being 1:0.1 to 1:1, and said hydrogen being contained in an amount of 20 to 67 atomic %.

#### BRIEF DESCRIPTION OF THE DRAWINGS

FIGS. 1 through 12 illustrate photosensitive members embodying the present invention in schematic cross sectional representation.

FIG. 13 illustrate examples of equipment for fabricating photosensitive members embodying the invention.

FIG. 14 is a schematic view of a resistance-heating type vapor deposition equipment for the preparation of a charge generating layer by vacuum vapor deposition.

FIG. 15 is a schematic view of a tester for the evaluation of a photosensitive member.

### DETAILED DESCRIPTION OF THE INVENTION

The present invention relates to a photosensitive member comprising:

an electrically conductive substrate;  
a charge generating layer; and

a charge transporting layer comprising amorphous carbon containing hydrogen, said amorphous carbon comprising hydrogen bonded carbon  $N_1$ , and carbon  $N_2$  free from linking with hydrogen, the ratio of the amount of  $N_1$  to that of  $N_2$  being 1:0.1 to 1:1, and said hydrogen being contained in an amount of 20 to 67 atomic %.

A photosensitive member of the invention comprising at least a charge generating layer and a charge transporting layer.

The charge transporting layer is composed of an amorphous carbon layer (a-C layer) containing hydrogen. The hydrogen content of the a-C layer is 20-67 atomic %, preferably 40-67 atomic %, most preferably 45-65 atomic %. If the hydrogen content is less than 20 atomic %, a sufficient transportability cannot be obtained, whereas being more than 67 atomic %, the properties and productivity of the a-C layer lower.

It is the characteristic of a photosensitive member of the invention that an a-C layer as a charge transporting layer is formed to have the ratio of hydrogen bonded carbon  $N_1$  and carbon  $N_2$  free from linking with hydrogen of from 1:0.1 to 1:1.

An a-C layer of the invention is suitable for a charge transporting layer when the value of  $N_2$  calculated as  $N_1$  being equal 1 is within the range of 0.1-1, preferably within the range of 0.2-0.8, most suitably within the range of 0.23-0.67. A photosensitive member constituted of the a-C layer having the value of less than 0.1 as the charge transporting layer has an increased electrical chargeability, but soon does not work as a photosensitive member because of charge up and the reduction of photosensitivity. If  $N_2$  is more than 1, the photosensitive member results in lower electrical chargeability and does not function as a photosensitive member.

The a-C layer of the present invention contains carbon atoms having various kinds of bond such as single bond (free radical), double bond or triple bond, and some of them are bonded with hydrogen and others are not bonded with hydrogen.

It is possible to determine whether the carbon atoms in the a-C layer have unsaturated bonds or not, and the number thereof may be analyzed either by an IR spectrum analysis, nuclear magnetic resonance by proton ( $^1H$ -NMR) or nuclear magnetic resonance by  $^{13}C$  ( $^{13}C$ -NMR) or combination thereof.

In the present invention an unsaturated bond means a double bond of carbon-carbon and/or a triple bond of carbon-carbon.

In the present invention, hydrogen bonded carbon  $N_1$  comprises unsaturated carbon  $N_3$  and saturated carbon  $N_4$ . And the objects of the invention is also achieved by forming an a-C layer as a charge transport-

ing layer wherein the ratio of said unsaturated carbon  $N_3$  and that of saturated carbon  $N_4$  is 1:1 to 1:16.

An a-C layer of the invention is suitable for a charge transporting layer when the value of  $N_4$  calculated as  $N_3$  being equal to 1 is within the range of 1-16, more preferably 1.2-1.4, and most suitably 1.5-7. The suitable transporting property is not attained if the value of  $N_4$  is more than 16. A photosensitive member constituted of an a-C layer having the value of more than 16 of  $N_4$  has

10 no photosensitivity and results in inadequacy in the injection of carrier and the transporting property. If the value of  $N_4$  is less than 1, unsaturated bonds (for example, double bonds of carbon) are generated in an a-C layer to excess, and that they work as trap-sites to deteriorate the transporting property of carrier. A photosensitive member constituted of the above layer has defects in not only inadequate charge voltage but also the increase of residual potential by the repetition of charge and exposure to light.

15 Generally, when the value of  $N_4$  is 1 or more, the specific resistance reaches approximately  $10^{11}$  ohms.cm or more and the mobility of the carrier increases to  $10^{-7}$  cm $^2$ /(V.sec.) or more with the result that a good transportability can be obtained.

20 In the present invention, carbon  $N_2$  free from linking with hydrogen comprises unsaturated carbon  $N_5$  and saturated carbon  $N_6$ , and the object of the invention is also achieved by forming an a-C layer as a charge transporting layer wherein the ratio of said unsaturated carbon  $N_5$  and that of saturated carbon  $N_6$  is 1:20 to 1:0.5.

25 An a-C layer of the invention is suitable for a charge transporting layer when the value of  $N_6$  calculated as  $N_5$  being equal to 1 is within the range of 0.5-20, more preferably 1-10, and most suitably 1.5-5. The suitable transporting property is not attained if the value of  $N_6$  is more than 20. A photosensitive member constituted of an a-C layer having the value of more than 20 of  $N_6$  has no photosensitivity and results in inadequacy in injection of carrier and transporting property. If the value of  $N_6$  is less than 0.5, unsaturated bonds (for example, double bonds of carbon) are generated in an a-C layer to excess, and that they work as trap-sites to deteriorate the transporting property of carrier. A photosensitive member constituted of the above layer has defects in not only inadequate charge voltage but also the increase of residual potential by the repetition of charge and exposure to light.

30 Generally, when the value of  $N_6$  is 0.5 or more, the specific resistance reaches approximately  $10^{11}$  ohms.cm or more and the mobility of the carrier increases to  $10^{-7}$  cm $^2$ /(V.sec.) or more.

35 In an a-C layer of the invention, there may exist therein various carbon atoms in various bonding manners. The number of all the carbon atoms in an a-C layer is obtained from the analyzed composition of the layer and its specific gravity. To wit, given  $C_xH_y(x+y=1)$  as the ratio of C to H in the analyzed composition of an organic plasma-polymerized layer and  $W(g/cm^3)$  as the specific gravity of the layer, the number of all the carbon atoms  $C_c$  contained in 1 cm $^3$  of the layer can be represented by the following equation [I]:

$$C_c = \frac{AW}{12x + y} \times (\text{per cm}^3) \quad [I]$$

wherein

$C_c$ : the number of all the carbon atoms

$W$ : specific gravity

x and y: ratios of the carbon and the hydrogen respectively in the analyzed composition

A: Avogadro's number (per mol).

In this invention, it is desirable that a part of the carbon atoms in an a-C layer free from linking with hydrogen has a ratio within the range of 5-65% based on all the carbon atoms therein.

The thickness suitable for an a-C layer ranges 5-50 microns, the preferable range being 7-20 microns. The surface potential is lower and the images can not be copied in a sufficient density if the thickness is below 5 microns, whereas the productivity is impaired if the thickness exceeds 50 microns. An a-C layer exhibits good transparency and a relatively high dark resistance, and has such a good charge transporting property that, even when the layer thickness exceeds 5 microns as described above, it transports the carrier without causing a charge trap.

Organic compounds for the production of a-C layer may not be always gas, but may be liquid or solid materials providing that the materials can be vaporized through melting, vaporization, sublimation, or the like when heated or vacuumed.

A hydrocarbon for this purpose can be selected from among, for example, methane series hydrocarbons, ethylene series hydrocarbons, acetylene series hydrocarbons, alicyclic hydrocarbons, aromatic hydrocarbons, etc. Further, these hydrocarbons can be mixed.

Examples of the methane series hydrocarbons applicable in this respect are:

normal-paraffins—methane, ethane, propane, butane, pentane, hexane, heptane, octane, nonane, decane, undecane, dodecane, tridecane, tetradecane, pentadecane, hexadecane, heptadecane, octadecane, nonadecane, eicosane, heneicosane, docosane, tricosane, tetracosane, pentacosane, hexacosane, heptacosane, octacosane, nonacosane, triacontane, dotriacontane, pentatriacontane, etc.; and

isoparaffins—isobutane, isopentane, neopentane, isohexane, neohexane, 2,3-dimethylbutane, 2-methylhexane, 3-ethylpentane, 2,2-dimethylpentane, 2,4-dimethylpentane, 3,3-dimethylpentane, triptane, 2-methylheptane, 3-methylheptane, 2,2-dimethylhexane, 2,2,5-dimethylhexane, 2,2,3-trimethylpentane, 2,2,4-trimethylpentane, 2,3,3-trimethylpentane, 2,3,4-trimethylpentane, isononane, etc.

Examples of the ethylene series hydrocarbons applicable in this respect are:

olefins—ethylene, propylene, isobutylene, 1-butene, 2-butene, 1-pentene, 2-pentene, 2-methyl-1-butene, 3-methyl-1-butene, 2-methyl-2-butene, 1-hexene, tetramethylethylene, 1-heptene, 1-octene, 1-nonene, 1-decene, etc.;

diolefins—allene, methylallene, butadiene, pentadiene, hexadiene, cyclopentadiene, etc.; and

triolefins—ocimene, allo-ocimene, myrcene, hexatriene, etc.

Examples of the acetylene series hydrocarbons applicable in this respect are:

acetylene, methylacetylene, 1-butyne, 2-butyne, 1-pentyne, 1-hexyne, 1-heptyne, 1-octyne, 1-nonyne, and 1-decyne.

Examples of the alicyclic hydrocarbons applicable in this respect are:

cycloparaffins—cyclopropane, cyclobutane, cyclopentane, cyclohexane, cycloheptane, cyclooctane, cyclononane, cyclodecane, cycloundecane, cyclodo-

decan, cyclotridecane, cyclotetradecane, cyclopentadecane, cyclohexadecane, etc.; cycloolefins—cyclopropene, cyclobutene, cyclopentene, cyclohexene, cycloheptene, cyclooctene, cyclononene, cyclodecene, etc.;

terpenes—limonene, terpinolene, phellandrene, silvestrene, thujene, carene, pinene, bornylene, camphene, fenchene, cyclofenchene, tricyclene, bisabolene, zingiberene, curcumene, humulene, cadine-sesquibenhen, selinene, caryophyllene, santalene, cedrene, camphorene, phyllocladene, podocarpene, mirene, etc.; and steroids.

Examples of the aromatic hydrocarbons applicable in this respect are:

benzene, toluene, xylene, hemimellitene, pseudocumene, mesitylene, prehnitene, isodurene, durene, pentamethyl benzene, hexamethyl benzene, ethylbenzene, propyl benzene, cumene, styrene, biphenyl, terphenyl, diphenylmethane, triphenylmethane, dibenzyl, stilbene, indene, naphthalene, tetralin, anthracene, and phenanthrene.

When the a-C layer is formed according to the present invention, two or more than two kinds of the above organic compounds may be co-used as a mixture. Various kinds of copolymer (block copolymer, graft copolymer and so on) are produced in the a-C layer so as to improve the hardness and adhesive property. If an alkane hydrocarbon ( $C_nH_{2n+2}$ ) is used, i-C layer, which has a Vickers hardness of not less than 2000, i.e.

25 diamond like supper hardness, and an electric resistance of  $10^9$  ohm.cm can be obtained. However, in this case as the plasma condition high temperature, lower pressure and high power must be employed with the application of direct bias to the substrate.

30 The carrier gases suitable in the practice of the invention are  $H_2$ ,  $Ar$ ,  $Ne$ ,  $He$ , etc.

In order to produce the a-C layer of the present invention various kinds of plasma method such as direct current, high frequency, low frequency or micro wave plasma method are applicable. As stated hereinafter the combination of an electromagnetic wave (X-ray, laser light etc.) with the plasma method is also applicable. According to the selection of the above methods various i-C layers different in properties can be obtained from the same monomer. For instance, using low frequency plasma method (frequency is from tens Hz to hundreds KHz), a-C layer having a high hardness can be obtained.

35 In the application of any of such processes, the most important thing for forming an a-C layer is that said a-C layer comprising hydrogen bonded carbon  $N_1$  and carbon  $N_2$  free from linking with hydrogen is constituted such that the ratio of the amount of  $N_1$  to that of  $N_2$  is 1:0.1 to 1:1.

40 Further, said hydrogen bonded carbon  $N_1$  comprises unsaturated carbon  $N_3$  and saturated carbon  $N_4$ , and it is preferable that the ratio of  $N_3$  to  $N_4$  is 1:1 to 1:16 in the present invention.

45 Moreover, said carbon  $N_2$  free from linking with hydrogen comprises unsaturated carbon  $N_5$  and saturated carbon  $N_6$ , and it is preferable that the ratio of  $N_5$  to  $N_6$  is 1:20 to 1:0.5 in the present invention.

In the case that the charge generating layer is formed by the high frequency plasma or P-CVD, a-C layer is 50 preferably formed by a method similar to the above in the aspect of device cost and process saving.

The charge generating layer of a photosensitive member according to the invention is not restricted to

any particular materials; the layer may be produced by, for example, amorphous silicon (a-Si) (which may contain hetero elements, e.g., H, C, O, S, N, P, B, a halogen, and Ge to change the property, and also may be a multi-layer), Se, Se-As, Se-Te, CdS, or a resin containing inorganic substances such as a copper phthalocyanine and zinc oxide and/or organic substances such as a bisazo pigment, triallylmethane dye, thiazine dye, oxazine dye, xanthene dye, cyanine colorant, styryl colorant, pyriliun dye, azo pigment, quinacridone pigment, indigo pigment, perylene pigment, polycyclic quinone pigment, bis-benzimidazole pigment, indanthrone pigment, squaleum pigment, and phthalocyanine pigment.

In the present invention phthalocyanine pigments may be used as charge generating materials. The phthalocyanines may be vapor depositable, and include monochloroaluminum monochlorophthalocyanine ( $AlClPc(Cl)$ ), titanyl phthalocyanine ( $TiOPc$ ), metal free phthalocyanine ( $H_2Pc$ ), aluminum monochlorophthalocyanine ( $AlClPc$ ), zinc phthalocyanine ( $ZnPc$ ), 20 magnesium phthalocyanine ( $MgPc$ ) and the like.

Inorganic compounds used as a charge generating materials may include  $Al_2O_3$ ,  $CaO$ ,  $CeO$ ,  $CeO_2$ ,  $CdO$ ,  $CoO$ ,  $Cr_2O_3$ ,  $CuO$ ,  $Cu_2O$ ,  $Fe_2O_3$ ,  $In_2O_3$ ,  $MgO$ ,  $MnO_2$ ,  $MoO_3$ ,  $NiO$ ,  $PbO$ ,  $SiO$ ,  $SiO_2$ ,  $SnO_2$ ,  $Ta_2O_5$ ,  $TiO$ ,  $TiO_2$ , 25  $Ti_2O_3$ ,  $WO_3$ ,  $Y_2O_3$ ,  $ZnO$ ,  $ZrO_2$ ,  $ZnS$ ,  $CdS$ ,  $CdSe$ ,  $CdTe$ ,  $PbS$ ,  $ZnSe$ ,  $MgF_2$  and the like.

More preferred inorganic materials are  $ZnS$ ,  $TiO_2$ ,  $ZnO$ ,  $Al_2O_3$ ,  $SiO$ ,  $SiO_2$ ,  $PbS$  etc.

In order to achieve the objects of the present invention more effectively,  $AlClPc(Cl)$ ,  $TiOPc$  or  $H_2Pc$  as phthalocyanine pigments, and  $ZnS$ ,  $Al_2O_3$  or  $SiO$  as an inorganic compounds may be used in combination. Examples of the most preferable combinations are  $AlClPc(Cl)$  with  $ZnS$ , and  $TiOPc$  with  $ZnS$ .

Besides the examples mentioned above, the charge generating layer may be of any material that is capable of absorbing light and generating a charge carrier with a very high efficiency.

The charge generating layer may be produced by a conventional method, for example, a method of coating a suitable binder resin dispersed with the powder of the above materials, plasma method and the like. If the charge transporting layer is formed by the plasma method, it is preferable to produce the charge generating layer by the plasma method because of the device costs and the process savings. In the case that the charge generating layer is produced by a conventional method, it is preferable to use the aforementioned inorganic materials, dyes or pigments which are previously coated with an organic material by plasma polymerization. When these inorganic materials, dye or pigments are dispersed in a resin, dispersibility, resistivity to a solvent, and prevention of spoilage will be achieved.

A charge generating layer according to the invention can be formed at any position in a photosensitive member, that is, for example, it can be formed at any of the top-most, intermediate and lowest layers. The thickness of the layer must in general be set such that a light of 550 nm can be absorbed 90% or more, though depended on the kind of the material used, especially its spectral absorption characteristic, light source for exposure, purpose, etc. With a-Si as the material the thickness must be within the range of 0.1-3 microns.

To adjust the charging property of an a-C charge transporting layer in invention, heteroatoms, other than carbon and hydrogen, can be incorporated into the material constituting said a-C charge transporting layer.

For example, to promote the transporting characteristic of the hole, atoms in Group III in the periodic table or halogen atoms can be incorporated. To promote the transporting characteristic of the electron, atoms in Group V in the periodic table or alkali metal atoms can be incorporated. To promote the transporting characteristic of both positive and negative carriers, atoms of Si, Ge, an alkali earth metal, or an chalcogen can be incorporated. These additive atoms can be used in a plurality of kinds together, at some specific positions in a charge transporting layer according to the purpose, can have a density gradient, or in some other specific manner, but whatever manner they may be added, it is essential to form an a-C polymer layer in which said a-C layer comprising hydrogen bonded carbon  $N_1$  and carbon  $N_2$  free from linking with hydrogen is constituted such that the ratio of the amount of  $N_1$  to that of  $N_2$  is 10:1 to 1:1.

In addition, it is preferable that carbon  $N_3$  linked with hydrogen and saturated carbon  $N_4$  linked with hydrogen in said a-C layer is constituted such that the ratio of the amount of  $N_3$  to that of  $N_4$  is 1:1 to 1:16, or unsaturated carbon  $N_5$  free from linking with hydrogen and saturated carbon  $N_6$  free from linking with hydrogen in said a-C layer is constituted such that the ratio of the amount of  $N_5$  to that of  $N_6$  is 1:20 to 1:0.5.

FIGS. 1 through 12 illustrate embodiments of the present invention, each in schematic sectional representation of models, wherein (1) denotes a substrate, (2) an a-C layer as a charge transporting layer, and (3) a charge generating layer. When a photosensitive member of the model shown in FIG. 1 is positively charged and then exposed to image light, a charge carrier is generated in the charge generating layer (3) and the electron neutralizes the surface charge while the positive hole is transported to the substrate (1) under guarantee of a good charge-transporting characteristic of the a-C layer (2). When the photosensitive member shown in FIG. 1 is negatively charged, contrarily the electron is transported through the a-C layer (2).

The photosensitive member illustrated in FIG. 2 is an example wherein an a-C layer (2) forms the topmost layer. When it is positively charged, the electron is transported through the a-C layer (2) and, when negatively charged, the hole is transported through the a-C layer (2).

FIG. 3 illustrates an embodiment of a photosensitive member of the present invention, in which on a substrate (1) a charge transporting layer (2), a charge generating layer (3) and then a charge transporting layer (2) are formed in this order.

FIGS. 4 through 6 illustrate the same photosensitive members as FIGS. 1 through 3, except that each additionally has a surfacc-protective overcoat (4) with thickness in the range of 0.01-5 microns, which, in keeping with the operating manner of the respective photosensitive member and the environment where it is used, is designed to protect the charge generating layer (3) or the charge transporting a-C layer (2) and to improve the initial surface potential as well. Any suitable material in public knowledge can be used to make the surface protective layers. It is desirable, in the practice of this invention, to make them by a technique of organic plasma polymerization from the viewpoint of manufacturing efficiency, etc. An a-C layer embodying the invention can also be used for this purpose. Heteroatoms, when required, can be incorporated into the protective layer (4).

FIGS. 7 through 9 illustrate the same photosensitive members as FIGS. 1 through 3, except that each additionally has an undercoat (5) with a thickness in the range of 0.01-5 microns which functions as an adhesion layer or a barrier layer. Depending on the substrate (1) or the process which it undergoes, this undercoat helps adhesion and prevents injection. Any suitable material in public knowledge can be used to make the undercoat. In this case, too, it is desirable to make them by a technique of organic plasma polymerization. An a-C layer according to the present invention can also be used for the purpose. The photosensitive members shown by FIGS. 7 through 9 can also be provided with an overcoat (4) as illustrated by FIGS. 4 through 6 (see FIGS. 10 through 12).

In the embodiments that the a-C layer is formed on the top surface as shown in FIGS. 2, 3, 8 or 9, the surface properties may be improved by the radiation of plasma of oxygen, hydrogen, inert gases, gases for a dry-etching (e.g. halogenized carbons) and/or nitrogen etc. By this treatment anti-moisture, resistance to rubbing and chargeability can be more improved.

A photosensitive member of the present invention has a charge generating layer and a charge transporting layer. Therefore the production requires at the least two processes. When, for example, an a-Si layer produced by equipment for glow discharge decomposition is used as the charge generating layer, the same vacuum equipment can be used for plasma polymerization, and it is naturally preferable in such cases to produce the a-C charge transporting layer, the surface-protective layer, the barrier layer, etc., by plasma polymerization.

It is preferable, in the present invention, that the charge transporting layer of the photosensitive member is produced by the so-called plasma-polymerizing reaction, that is, for example:

molecules in the vapor phase undergo discharge decomposition under reduced pressure and produce a plasma atmosphere, from which active neutral seeds or charged seeds are collected on the substrate by diffusing, electrical or magnetic guiding, etc. and deposited as a solid on the substrate through recombination reaction

FIG. 13 illustrates an equipment for the production of a photosensitive member of the present invention, which is a capacitive coupling type plasma CVD equipment. Exemplifying a photosensitive member having a plasma polymerized polyethylene layer as a charge transporting layer, the production thereof is explained according to FIG. 13.

In FIG. 13, the numerals (701)-(706) denote No. 1 tank through No. 6 tank which are filled with a feedstock (a compound in the vapor phase at normal temperatures) and a carrier gas, each tank connected with one of six regulating valves No. 1 through No. 6 (707)-(712) and one of six flow controllers No. 1 through No. 6 (713)-(718).

(719)-(721) show vessels No. 1 through No. 3 which contain a feedstock which is a compound either in the liquid phase or in the solid phase at normal temperatures, each vessel being capable of being heated for vaporization by means of one of three heaters No. 1 through No. 3 (722)-(724) to the temperature of, for example, from the room temperature to 150° C. or from -50° C. to the room temperature. Each vessel is connected with one of three regulating valves No. 7 through No. 9 (725)-(727) and also with one of three flow controllers No. 7 through No. 9 (728)-(730).

These gases are mixed in a mixer (731) and sent through a main pipe (732) into a reactor (733). The piping is equipped at intervals with pipe heaters (734) so that the gases that are vaporized forms of the feedstock compounds in the liquid or solid state at normal temperatures are prevented from condensing or congealing in the pipes.

In the reaction chamber, there are a grounding electrode (735) and a power-applying electrode (736) installed oppositely, each electrode with a heater (737) for heating the electrode.

Said power-applying electrode is connected to a high frequency power source (739) with a matching box (738) for high frequency power interposed in the connection circuit, to a low frequency power source (741) likewise with a matching box (740) for low frequency power, and to a direct current power source (743) with a low-pass filter (742) interposed in the connection circuit, so that by a connection-selecting switch (744) the mechanism permits application of electric power with a different frequency.

The pressure in the reaction chamber can be adjusted by a pressure control valve (745), and the reduction of the pressure in the reaction chamber can be carried out through an exhaust system selecting valve (746) and by operating a diffusion pump (747) and an oil-sealed rotary vacuum pump (748) in combination or by operating a cooling-elimination device (749), a mechanical booster pump (750) and an oil-sealed rotary vacuum pump in combination.

The exhaust gas is discharged into the ambient air after conversion to a safe unharful gas by a proper elimination device (753).

The piping in the exhaust system, too, is equipped with pipe heaters at intervals in the pipe lines so that the gases which are vaporized forms of feedstock compounds in the liquid or solid state at normal temperatures are prevented from condensing or congealing in the pipes.

For the same reason the reaction chamber, too, is equipped with a heater (751) for heating the chamber, and an electrode therein are provided with a conductive substrate (752) for the purpose.

FIG. 13 illustrates a conductive substrate (752) fixed to a grounding electrode (735), but it may be fixed to the power-applying electrode (736) and to both the electrodes as well.

The reaction chamber for the production of a photosensitive member is preliminarily decreased to a level in the range of about  $10^{-4}$  to  $10^{-6}$  Torr by the diffusion pump, the degree of vacuum is checked, and then the gas absorbed inside the equipment is removed. Simultaneously, by the heater for electrode, the electrode and the conductive substrate fixed to the opposing electrode are heated to a given temperature.

Then, from six tanks, No. 1 through No. 6, and from three vessels, No. 1 through No. 3, gases of the raw materials are led into the reaction chamber by regulating the gas flows at constant rates using the nine flow controllers, No. 1 through No. 9 and simultaneously the pressure in the reaction chamber is reduced constantly to a specified level by a pressure regulating valve.

After the gas flows have stabilized, the connection-selecting switch is put in position for, for example, the high frequency power source so that high frequency power is supplied to the power-applying electrode. An electrical discharge begins between the two electrodes

and an a-C layer in the solid state is formed on the conductive substrate with time.

In the above constitution, for example, when the photosensitive member shown in FIG. 1 is produced, after the reaction chamber (733) is controlled to a given vacuum state,  $C_2H_4$  gas from No. 1 tank (701) and  $H_2$  gas as carrier gas from No. 2 tank (702) are supplied through the gas line (732). On the other hand, an electric power (e.g. 10 watts-1K watts) is applied to the upper electrode (736) through the high frequency power source (739) to cause plasma discharge between the two electrodes to form the a-C charge transporting layer (2) having a thickness of 5 to 50 micron meter on a previously heated Al substrate plate (752). The ratio of the amount of hydrogen bonded carbon  $N_1$  to the amount of carbon  $N_2$  free from linking with hydrogen can be controlled, being dependent upon the conditions of the production, such as the electric power, the electric power frequency, the space between the electrodes, the pressure, the temperature of the substrate, kinds of the gases used as feedstock, concentrations of such gases, and flow rates of such gases. For example, the ratio of  $N_1$  to  $N_2$  within the range of 1:0.1 to 1:1 can be controlled by application of bias voltages in the range of 10 V-1 KV supplied from the direct current power source (743) being dependent on other conditions.

The higher bias voltage is applied, the less hydrogen bonded carbon is generated for an a-C layer to get to have more hardness.

The ratio of the amount of the unsaturated carbon  $N_3$  linked with hydrogen to the amount of saturated carbon  $N_4$  linked with hydrogen within the range of 1:1-1:16 and the ratio of the amount of the unsaturated carbon  $N_5$  free from linking with hydrogen to the amount of saturated carbon  $N_6$  free from linking with hydrogen within the range of 1:20-1:0.5 are also controlled as above-mentioned. That is, the higher bias voltage is applied, the less unsaturated carbon linked with hydrogen and unsaturated carbon free from linking with hydrogen are generated and an a-C layer gets to have more hardness.

The a-C charge transporting layer formed by the above process is excellent in a transmittance, a dark resistance, and a transportability of charge carrier remarkably. The polarity of this layer may be controlled to P or N type by introducing  $B_2H_6$  gas from No. 4 tank (704) or  $PH_3$  gas from No. 5 tank (705) to increase the charge transportability.

The charge generating layer (3) may be produced by introducing  $H_2$  gas from No. 2 tank (702) and  $SiH_4$  gas from No. 3 tank (703) as a layer essentially consisting of a-Si.

When the compounds introduced into the reaction chamber (733) for the formation of a charge transporting layer is a liquid material, the gas may be introduced into the chamber (733) to cause plasma-polymerization as described above.

In the case that the a-C layer is made from organic compounds having a high boiling point, these compounds are previously coated on the surface of the substrate, and then plasma of a carrier gas or others are irradiated on the substrate to polymerize then (so-called plasma-polymerization).

In the plasma-polymerization of a-C layer of the present invention electromagnetic wave such as laser beam, ultraviolet ray, X-ray or electron beam may be irradiated alone or as a supplement (photo-assist method), or the assistance of magnetic field or bias direct electric

field may be effectively used. The photo-assist method is effective to quicken the deposition rate of the a-C layer, to shorten the production time and to increase the hardness of the a-C layer.

FIG. 14 is a schematic view of a resistance-heating type vapor deposition equipment for a preparation of a charge generation layer by a vacuum vapor deposition.

The equipment includes vacuum chamber (101), substrate holder (102), substrate (103), shutter (104), boats (105) and (106), outlet (107) and electrodes (108).

The charge generating layer of the present invention may be made by the following processes.

The boats (105) and (106) which contain phthalocyanine pigments and inorganic compounds respectively are set up to the electrodes (108), and the substrate (103) is to the substrate holder (102). The vacuum chamber (101) is vacuumed through the outlet (107) by a vacuum pump (not illustrated in FIG. 14). The amount of the materials deposited on the substrate (103) from the boats (105) and (106) can be controlled by the shutter (104). A shield (not shown in FIG. 14) may be provided between the boats (105) and (106) to prevent the mutual influence of the temperature of the each boat.

The condition of the vapor deposition such as the degree of the vacuum pressure, boat temperature, evaporation time, amount of pigments and inorganic compounds and others may be selected according to a variation of a charge generating layer, a thickness of thereof, a ratio of the pigments to the inorganic compounds and others for a desired charge generating layer.

A charge generating layer and a charge transporting layer can be continuously formed by incorporating a vapor deposition equipment as shown in FIG. 14 into a glow discharge decomposition equipment as shown in FIG. 13.

Though the main application of the a-C layer of the present invention is to a charge transporting layer as aforementioned, the a-C layer of the present invention may be used for an overcoat layer having a charge transportability. Even in the case that the a-C layer of the present invention is applied to an overcoat layer alone, an excellent durability, of course, can be achieved without increase of residual potential.

This invention will now be explained with reference to examples hereunder.

#### EXAMPLE 1

##### (I) Formation of an a-C Layer:

In a system of glow discharge decomposition with equipment as illustrated in FIG. 13, first the reaction chamber (733) was vacuumized inside to a high level of approximately  $10^{-6}$  Torr, and then by opening No. 1 and No. 2 regulating valves (707) and (708),  $C_2H_4$  gas from No. 1 tank (701) and  $H_2$  gas from No. 2 tank (702) were led, under output pressure gage reading of 1  $Kg/cm^2$ , into mass flow controllers (713) and (714). Then, the mass flow controllers were set so as to make  $C_2H_4$  flow at 40 sccm and  $H_2$  flow at 70 sccm, and the gases were allowed into the reaction chamber (733). After the respective flows had stabilized, the internal pressure of the reaction chamber (733) was adjusted to 0.5 Torr. On the other hand, the electrically conductive substrate (752), which was an aluminum plate of  $2 \times 50 \times 50$  mm, was preliminarily heated up to  $240^\circ C$ , and while the gas flows and the internal pressure were stabilized, it was connected to the high frequency power source (739) and 80 watts power (frequency:

13.56 MHz) was applied to the power-applying electrode (736). After plasma polymerization for approximately four hours, there was formed a charge transporting layer constituted of plasma-polymerized ethylene layer with a thickness of approximately 6.0 microns on the conductive substrate (752).

The resultant plasma-polymerized ethylene layer is analyzed with the Fourier transform infrared absorption spectroscope (made by Perkin Elmer Ltd.), the <sup>13</sup>C-NMR system (solid-NMR, made by Nippon Densi Ltd.) and the <sup>1</sup>H-NMR system (made by Nippon Densi Ltd.). In the chemical structure of the plasma-polymerized ethylene layer, the ratio N<sub>1</sub>:N<sub>2</sub>) of the amount of hydrogen-bonded carbon N<sub>1</sub> to that of carbon N<sub>2</sub> free from linking with hydrogen was about 80:20, namely 1:0.2. The above layer had  $3 \times 10^{12} \Omega \cdot \text{cm}$  or less of dark specific resistance and 10<sup>2</sup>-10<sup>4</sup> or more of the ratio of the dark specific resistance to the light specific resistance. The plasma-polymerized ethylene layer of the invention has been found to be applied effectively to a photosensitive member.

#### (II) Formation of a charge generating layer:

The power application from the high frequency power source (739) was stopped for a time and the reaction chamber was vacuumized inside.

By opening No. 3 and No. 2 regulating valves (709) and (708), SiH<sub>4</sub> gas from No. 3 tank (703) and H<sub>2</sub> gas from No. 2 tank (702) were, under output pressure gage reading of 1 Kg/cm<sup>2</sup>, led into the mass flow controllers (715) and (714). Then, the mass flow controllers were set so as to make SiH<sub>4</sub> flow at 90 sccm and H<sub>2</sub> flow at 210 sccm, and the gases were allowed into the reaction chamber. After the respective flows had stabilized, the internal pressure of the reaction chamber (733) was adjusted to 1.0 Torr.

While the gas flows and the internal pressure were stabilized, the circuit to the high frequency power source (739) was supplied and a 30 W power (frequency: 13.56 MHz) was applied to the power-applying electrode (736) to generate glow discharge. After 10 minutes of glow discharge, there was formed an a-Si:H charge generating layer with a thickness of 1 micron.

#### (III) Test of property of photosensitive member:

The photosensitive member produced according to the above processes (I) and (II) was evaluated in its chargeability and sensitivity using the tester for a photosensitive member as illustrated in FIG. 15.

The sample of the photosensitive member produced (35) was put on the scanning table (37), and fixed by the shield cover (36). The scanning table (37) was moved to the charged area (52), and a high electric power supplied from the direct high electric power (40) of +7.7 KV was applied to the charger (42) to generate corona discharge on the surface of the photosensitive member, and then the scanning table (37) was moved to the discharge area (51). The surface potential of the corona discharged sample was sensed by the transparent electrode (48) to be indicated on the surface potential meter (49), and then put out on the recorder (50). The photosensitive member of the above showed an excellent chargeability.

Further, the shutter (47) was opened to irradiate the light from the halogen lamp (43), which was reflected on the mirror (44), on the surface of the charged sample (35). The irradiation was effected through the transparent electrode (48), and the change of the surface poten-

tial by the irradiation was put out on the recorder (50) as well as the electric current at the same time was sensed by the photo-electric current monitor (38). The photosensitive member of the above showed a half-reduced exposure value E<sub>1</sub> of about 0.8 lux.sec for an initial surface potential (V<sub>0</sub>) of -490 volt.

Furthermore, a drum type of a photosensitive member was made in the same manner as the Example 1 excepting that the electric power of 250 W, the flow ratio of C<sub>2</sub>H<sub>4</sub> of 300 sccm, and the flow ratio of H<sub>2</sub> of 650 sccm were used as the condition of the production for the charge transporting layer, and the electric power of 250 W, SiH<sub>4</sub> of 180 sccm and H<sub>2</sub> of 500 sccm were used as the condition for the charge generating layer and assembled into the copying machine (EP-650Z) produced by Minolta Kamera K.k. to be tested for the image transfer. The obtained images were excellent.

A simulation test for a copying process was made using a tester of drum type photosensitive member (not shown). There was obtained a stable static electric property even after the repeat of 50000 times of full copying process (charge - exposure - transferring and charge for removal - erasing).

## EXAMPLE 2

(I) In a system of glow discharge decomposition with equipment as illustrated in FIG. 13, first the reaction chamber (733) was vacuumized inside to a high level of approximately 10<sup>-6</sup> Torr, and then by opening No. 1 and No. 2 regulating valves (707) and (708), C<sub>2</sub>H<sub>2</sub> gas from No. 1 tank (701) and H<sub>2</sub> gas from No. 2 tank (702) were led, under output pressure gage reading of 1 Kg/cm<sup>2</sup>, into mass flow controllers (713) and (714). Then, the mass flow controllers were set so as to make C<sub>2</sub>H<sub>2</sub> flow at 70 sccm and H<sub>2</sub> flow at 80 sccm, and the gases were allowed into the reaction chamber (733). After the respective flows had stabilized, the internal pressure of the reaction chamber (733) was adjusted to 1.0 Torr. On the other hand, the electrically conductive substrate (752), which was a aluminium plate of 2×50×50 mm, was preliminarily heated up to 200° C., and while the gas flows and the internal pressure were stabilized, it was connected to the high frequency power source (739) and 85 watts power (frequency: 13.56 MHz) was applied to the power-applying electrode (736). After plasma polymerization for approximately 1.6 hours, there was formed a charge transporting layer with a thickness of approximately 9 microns on the conductive substrate (752).

The ratio of N<sub>1</sub> to N<sub>2</sub> N<sub>1</sub>:N<sub>2</sub>) in the charge transporting layer was about 63:37, namely 1:0.59.

#### (II) Formation of a charge generating layer:

The power application from the high frequency power source (739) was stopped for a time and the reaction chamber was vacuumized inside

By opening No. 4 and No. 2 regulating valves (710) and (708), SiH<sub>4</sub> gas from No. 4 tank (704) and H<sub>2</sub> gas from No. 2 tank (702) were, under output pressure gage reading of 1 Kg/cm<sup>2</sup>, led into the mass flow controllers (716) and (714). Then, the mass flow controllers were set so as to make SiH<sub>4</sub> flow at 90 sccm and H<sub>2</sub> flow at 210 sccm, and the gases were allowed into the reaction chamber. After the respective flows had stabilized, the internal pressure of the reaction chamber (733) was adjusted to 1.0 Torr.

While the gas flows and the internal pressure were stabilized, the circuit to the high frequency power source (739) was supplied and a 30 W power (frequency: 13.56 MHz) was applied to the power-applying electrode (736) to generate glow discharge. After 10 minutes of glow discharge, there was formed an a-Si:H charge generating layer with a thickness of 1 micron.

The photosensitive member thus obtained showed a half-reduced exposure value  $E_{1/2}$  of 0.5 lux.sec for the initial surface potential ( $V_0$ ) = -480 volt. This photosensitive member, tested for the image transfer, produced clear images.

### EXAMPLE 3

(I) In a system of glow discharge decomposition with equipment as illustrated in FIG. 13, first the reaction chamber (733) was vacuumized inside to a high level of approximately  $10^{-6}$  Torr, and then by opening No. 1-No. 3 regulating valves (707)-(709),  $C_2H_4$  gas from No. 1 tank (701),  $CH_4$  gas from No. 2 tank (702) and  $H_2$  gas from No. 3 tank (703) were led, under output pressure gage reading of 1  $Kg/cm^2$ , into mass flow controllers (713)-(715). Then, the mass flow controllers were set so as to make  $C_2H_4$  flow at 50 sccm,  $CH_4$  flow at 100 sccm, and  $H_2$  flow at 120 sccm, and the gases were allowed into the reaction chamber (733). After the respective flows had stabilized, the internal pressure of the reaction chamber (733) was adjusted to 1.0 Torr. On the other hand, the electrically conductive substrate (752), which was an aluminum plate of  $2 \times 50 \times 50$  mm, was preliminarily heated up to  $250^\circ C$ , and while the gas flows and the internal pressure were stabilized, it was connected to the high frequency power source (739) and 200 watts power (frequency: 13.56 MHz) was applied to the power-applying electrode (736). After plasma polymerization for approximately 5 hours, there was formed a charge transporting layer with a thickness of approximately 5.9 microns on the conductive substrate (752).

The ratio of  $N_1$  to  $N_2$  ( $N_1:N_2$ ) in the charge transporting layer was 82:18, namely 1:0.22.

And then an a-Si charge generating layer was formed on the charge transporting layer obtained in the above process in a similar way as example 2 (II).

The photosensitive member thus obtained showed a half-reduced exposure value  $E_{1/2}$  of 1.5 lux.sec for the initial surface potential ( $V_0$ ) = -520 volt. This photosensitive member, tested for the image transfer, produced clear images.

### EXAMPLE 4

(I) In a system of glow discharge decomposition with equipment as illustrated in FIG. 13, first the reaction chamber (733) was vacuumized inside to a high level of approximately  $10^{-6}$  Torr, and then by opening No. 1-No. 3 regulating valves (707)-(709),  $C_2H_4$  gas from No. 1 tank (701),  $CH_4$  gas from No. 2 tank (702) and  $H_2$  gas from No. 3 tank (703) were led, under output pressure gage reading of 1  $Kg/cm^2$ , into mass flow controllers (713)-(715). Then, the mass flow controllers were set so as to make  $C_2H_4$  flow at 55 sccm,  $CH_4$  flows at 60 sccm and  $H_2$  flow at 100 sccm, and the gases were allowed into the reaction chamber (733). After the respective flows had stabilized, the internal pressure of the reaction chamber (733) was adjusted to 2.0 Torr. On the other hand, the electrically conductive substrate (752), which was an aluminum plate of  $2 \times 50 \times 50$  mm, was preliminarily heated up to  $250^\circ C$ , and while the

gas flows and the internal pressure were stabilized, it was connected to the high frequency power source (739) and 200 watts power (frequency: 13.56 MHz) was applied to the power-applying electrode (736). After plasma polymerization for approximately 4.5 hours, there was formed a charge transporting layer with a thickness of approximately 5 microns on the conductive substrate (752).

The ratio of  $N_1$  to  $N_2$  ( $N_1:N_2$ ) in the charge transporting layer was about 58:42, namely 1:0.72.

And then an a-Si charge generating layer was formed on the charge transporting layer obtained in the above process in a similar way as example 2 (II).

The photosensitive member thus obtained showed a half-reduced exposure value  $E_{1/2}$  of about 1.8 lux.sec for the initial surface potential ( $V_0$ ) = -540 volt. This photosensitive member, tested for the image transfer, produced clear images.

### EXAMPLE 5

In a system of glow discharge decomposition with equipment as illustrated in FIG. 13, first the reaction chamber (733) was vacuumized inside to a high level of approximately  $10^{-6}$  Torr, and then by opening No. 6 and No. 7 regulating valves (712) and (725),  $H_2$  gas from No. 6 tank (706) and styrene gas from No. 1 vessel (719) heated at the temperature of about  $20^\circ C$ . by No. 1 heater (722), were led, under output pressure gage reading of 1  $Kg/cm^2$ , into mass flow controllers (718) and (728). Then, the mass flow controllers were set so as to make  $H_2$  flow at 30 sccm and styrene ( $C_9H_8$ ) flow at 60 sccm, and the gases were allowed into the reaction chamber (733). After the respective flows had stabilized, the internal pressure of the reaction chamber (733) was adjusted to 0.4 Torr. On the other hand, the electrically conductive substrate (752), which was an aluminum plate of  $2 \times 50 \times 50$  mm, was preliminarily heated up to  $150^\circ C$ , and while the gas flows and the internal pressure were stabilized, it was connected to the low frequency power source (741) and 120 watts power (frequency: 30 KHz) was applied to the power-applying electrode (736). After plasma polymerization for approximately 40 minutes, there was formed a charge transporting layer with a thickness of approximately 9 microns on the conductive substrate (752).

The ratio of  $N_1$  to  $N_2$  in the charge transporting layer was 54:46, namely 1:0.85.

And then an a-Si generating layer was formed on the charge transporting layer obtained in the above process in a similar way as Example 2 (II).

The photosensitive member thus obtained showed a half-reduced exposure value  $E_{1/2}$  of 4 lux.sec for the initial surface potential ( $V_0$ ) = -670 volt. This photosensitive member had a practicable sensitivity, and tested for the image transfer, produced clear images.

### EXAMPLE 6

Using the vapor deposition equipment of FIG. 14, titanylphthalocyanine was codeposited on an aluminum substrate under a vaccum of not more than  $1 \times 10^{-5}$  Torr, and the boat temperature of  $400^\circ$ - $600^\circ C$ , at the same time  $ZnS$  was deposited under the boat temperature  $900^\circ$ - $1150^\circ C$ . The resultant codeposited layer had a thickness of 1000 Å.

Then, an a-C layer as a charge transporting layer was formed thereon with the same method as Example 5.

The ratio (N<sub>1</sub>:N<sub>2</sub>) of the obtained layer of the amount of hydrogen bonded carbon N<sub>1</sub> to that of carbon N<sub>2</sub> free from linking with hydrogen was 1:0.6.

The photosensitive member obtained above showed a half-reduced exposure value E<sub>1</sub> of 6.0 lux.sec for the initial surface potential (V<sub>0</sub>) of +550 V.

Further, this member showed a half-reduced exposure value E<sub>1</sub> of 15.4 erg/cm<sup>2</sup> toward the semiconductor laser light having a wave length of 780 nm.

Moreover, a photosensitive member was prepared to form the a-C layer of Example 6 on a charge generating layer made of non-crystal Se-Te or Se-As, each charge generating layer having a thickness of 1.2  $\mu$ m. The photosensitive members thus obtained showed excellent electrophotographic properties.

#### EXAMPLE 7

##### (I) Formation of an a-C Layer:

In a system of glow discharge decomposition with equipment as illustrated in FIG. 13, first the reaction chamber (733) was vacuumized inside to a high level of approximately 10<sup>-6</sup> Torr, and then by opening No. 1 and No. 2 regulating valves (707) and (708), C<sub>2</sub>H<sub>4</sub> gas from No. 1 tank (701) and H<sub>2</sub> gas from No. 2 tank (702) were led, under output pressure gage reading of 1 Kg/cm<sup>2</sup>, into mass flow controllers (713) and (714). Then, the mass flow controllers were set so as to make C<sub>2</sub>H<sub>4</sub> flow at 30 sccm and H<sub>2</sub> flow at 50 sccm, and the gases were allowed into the reaction chamber (733). After the respective flows had stabilized, the internal pressure of the reaction chamber (733) was adjusted to 0.5 Torr. On the other hand, the electrically conductive substrate (752), which was an aluminum plate of 2×50×50 mm, was preliminarily heated up to 250° C., and while the gas flows and the internal pressure were stabilized, it was connected to the high frequency power source (739) and 100 watts power (frequency: 13.56 MHz) was applied to the power-applying electrode (736). After plasma polymerization for approximately 3.5 hours, there was formed a charge transporting layer with a thickness of approximately 6 microns on the conductive substrate (752).

The resultant plasma-polymerized ethylene layer is analyzed with the Fourier transform infrared absorption spectroscope (made by Perkin Elmer Ltd.), the <sup>13</sup>C-NMR system (solid-NMR, made by Nippon Densi Ltd.) and the <sup>1</sup>H-NMR system (made by Nippon Densi Ltd.). In the chemical structure of the plasma-polymerized ethylene layer, the ratio (N<sub>3</sub>:N<sub>4</sub>) of the amount of unsaturated carbon N<sub>3</sub> linked with hydrogen to that of saturated carbon N<sub>4</sub> linked with hydrogen was approximately 1:5. The above layer had  $2.5 \times 10^{14}$   $\Omega$ .cm or less of the dark specific resistance and 10<sup>2</sup>–10<sup>4</sup> or more of the ratio of the dark specific resistance to the light specific resistance. The plasma-polymerized ethylene layer of the invention has been found to be applied effectively to a photosensitive member.

##### (II) Formation of a charge generating layer:

The power application from the high frequency power source (739) was stopped for a time and the reaction chamber was vacuumized inside.

By opening No. 3 and No. 2 regulating valves (709) and (708), SiH<sub>4</sub> gas from No. 3 tank (703) and H<sub>2</sub> gas from No. 2 tank (702) were, under output pressure gage reading of 1 Kg/cm<sup>2</sup>, led into the mass flow controllers (715) and (714). Then, the mass flow controllers were set so as to make SiH<sub>4</sub> flow at 90 sccm and H<sub>2</sub> flow at

210 sccm, and the gases were allowed into the reaction chamber. After the respective flows had stabilized, the internal pressure of the reaction chamber (733) was adjusted to 1.0 Torr.

While the gas flows and the internal pressure were stabilized, the circuit to the high frequency power source (739) was supplied and a 30 W power (frequency: 13.56 MHz) was applied to the power-applying electrode (736) to generate glow discharge. After 10 minutes of glow discharge, there was formed an a-Si:H charge generating layer with a thickness of 1 micron.

##### (III) Test of property of photosensitive member:

The photosensitive member produced according to the above processes (I) and (II) was evaluated in its chargeability and sensitivity using the tester for a photosensitive member as illustrated in FIG. 15.

The sample of the photosensitive member produced (35) was put on the scanning table (37), and fixed by the shield cover (36). The scanning table (37) was moved to the charged area (52), and a high electric power supplied from the direct high electric power (40) of +7.7 KV was applied to the charger (42) to generate corona discharge on the surface of the photosensitive member, and then the scanning table (37) was moved to the discharge area (51). The surface potential of the corona discharged sample was sensed by the transparent electrode (48) to be indicated on the surface potential meter (49), and then put out on the recorder (50). The photosensitive member of the above showed an excellent chargeability.

Further, the shutter (47) was opened to irradiate the light from the halogen lamp (43), which was reflected on the mirror (44), on the surface of the charged sample (35). The irradiation was effected through the transparent electrode (48), and the change of the surface potential by the irradiation was put out on the recorder (50) as well as the electric current at the same time was sensed by the photo-electric current monitor (38). The photosensitive member of the above showed a half-reduced exposure value E<sub>1</sub> of about 0.7 lux.sec for an initial surface potential (V<sub>0</sub>) of -510 volt.

Furthermore, a drum type of a photosensitive member was made in the same manner as the Example 1 excepting that the electric power of 250 W, the flow ratio of C<sub>2</sub>H<sub>4</sub> of 300 sccm, and the flow ratio of H<sub>2</sub> of 600 sccm were used as the condition of the production for the charge transporting layer, and the electric power of 250 W, SiH<sub>4</sub> of 180 sccm and H<sub>2</sub> of 500 sccm were used as the condition for the charge generating layer and assembled into the copying machine (EP-650Z) produced by Minolta Kamera K.k. to be tested for the image transfer. The obtained images were excellent.

A simulation test for a copying process was made using a tester of drum type photosensitive member (not shown). There was obtained a stable static electric property even after the repeat of 50000 times of full copying process (charge - exposure - transferring and charge for removal - erasing).

#### EXAMPLE 8

##### (I) Formation of an a-C Layer:

In a system of glow discharge decomposition with equipment as illustrated in FIG. 13, first the reaction chamber (733) was vacuumized inside to a high level of approximately 10<sup>-6</sup> Torr, and then by opening No. 1

and No. 2 regulating valves (707) and (708),  $C_2H_2$  gas from No. 1 tank (701) and  $H_2$  gas from No. 2 tank (702) were led, under output pressure gage reading of 1  $Kg/cm^2$ , into mass flow controllers (713) and (714). Then, the mass flow controllers were set so as to make  $C_2H_2$  flow at 60 sccm and  $H_2$  flow at 80 sccm, and the gases were allowed into the reaction chamber (733). After the respective flows had stabilized, the internal pressure of the reaction chamber (733) was adjusted to 0.8 Torr. On the other hand, the electrically conductive substrate (752), which was a aluminum plate of  $2 \times 50 \times 50$  mm, was preliminarily heated up to  $200^\circ C$ , and while the gas flows and the internal pressure were stabilized, it was connected to the high frequency power source (739) and 85 watts power (frequency: 13.56 MHz) was applied to the power-applying electrode (736). After plasma polymerization for approximately 1.2 hours, there was formed a charge transporting layer with a thickness of approximately 10 microns on the conductive substrate (752).

The ratio ( $N_3:N_4$ ) of  $N_3$  to  $N_4$  in the charge transporting layer was about 20:36, namely 1:1.8.

#### (II) Formation of a charge generating layer:

The power application from the high frequency power source (739) was stopped for a time and the reaction chamber was vacuumized inside.

By opening No. 4 and No. 2 regulating valves (710) and (708),  $SiH_4$  gas from No. 4 tank (704) and  $H_2$  gas from No. 2 tank (702) were, under output pressure gage reading of 1  $Kg/cm^2$ , led into the mass flow controllers (716) and (714). Then, the mass flow controllers were set so as to make  $SiH_4$  flow at 90 sccm and  $H_2$  flow at 210 sccm, and the gases were allowed into the reaction chamber. After the respective flows had stabilized, the internal pressure of the reaction chamber (733) was adjusted to 1.0 Torr.

While the gas flows and the internal pressure were stabilized, the circuit to the high frequency power source (739) was supplied and a 30 W power (frequency: 13.56 MHz) was applied to the power-applying electrode (736) to generate glow discharge. After 10 minutes of glow discharge, there was formed an a-Si:H charge generating layer with a thickness of 1 micron.

The photosensitive member thus obtained showed a half-reduced exposure value  $E_1$  of 0.5 lux.sec for the initial surface potential ( $V_0$ ) = -460 volt. This photosensitive member, tested for the image transfer, produced clear images.

#### EXAMPLE 9

(I) In a system of glow discharge decomposition with equipment as illustrated in FIG. 13, first the reaction chamber (733) was vacuumized inside to a high level of approximately  $10^{-6}$  Torr, and then by opening No. 1-No. 3 regulating valves (707)-(709),  $C_2H_2$  gas from No. 1 tank (701),  $CH_4$  gas from No. 2 tank (702) and  $H_2$  gas from No. 3 tank (703) were led, under output pressure gage reading of 1  $Kg/cm^2$ , into mass flow controllers (713)-(715). Then, the mass flow controllers were set so as to make  $C_2H_2$  flow at 50 sccm,  $CH_4$  flow at 100 sccm, and  $H_2$  flow at 100 sccm, and the gases were allowed into the reaction chamber (733). After the respective flows had stabilized, the internal pressure of the reaction chamber (733) was adjusted to 1.0 Torr. On the other hand, the electrically conductive substrate (752), which was an aluminum plate of  $2 \times 50 \times 50$  mm, was preliminarily heated up to  $250^\circ C$ , and while the

gas flows and the internal pressure were stabilized, it was connected to the high frequency power source (739) and 200 watts power (frequency: 13.56 MHz) was applied to the power-applying electrode (736). After 5 plasma polymerization for approximately 5 hours, there was formed a charge transporting layer with a thickness of approximately 7 microns on the conductive substrate (752).

The ratio of  $N_3$  to  $N_4$  ( $N_3:N_4$ ) in the charge transporting layer was 7:78, namely 1:11.1.

And then an a-Si charge generating layer was formed on the charge transporting layer obtained in the above process in a similar way as Example 8(II).

The photosensitive member thus obtained showed a half-reduced exposure value  $E_1$  of 1.3 lux.sec for the initial surface potential ( $V_0$ ) = -510 volt. This photosensitive member, tested for the image transfer, produced clear images.

#### EXAMPLE 10

(I) In a system of glow discharge decomposition with equipment as illustrated in FIG. 13, first the reaction chamber (733) was vacuumized inside to a high level of approximately  $10^{-6}$  Torr, and then by opening No. 1-No. 3 regulating valves (707)-(709),  $C_2H_4$  gas from No. 1 tank (701),  $CH_4$  gas from No. 2 tank (702) and  $H_2$  gas from No. 3 tank (703) were led, under output pressure gage reading of 1  $Kg/cm^2$ , into mass flow controllers (713)-(715). Then, the mass flow controllers were set so as to make  $C_2H_4$  flow at 65 sccm,  $CH_4$  gas flows at 50 sccm and  $H_2$  flow at 100 sccm, and the gases were allowed into the reaction chamber (733). After the respective flows had stabilized, the internal pressure of the reaction chamber (733) was adjusted to 1.5 Torr. On the other hand, the electrically conductive substrate (752), which was an aluminum plate of  $2 \times 50 \times 50$  mm, was preliminarily heated up to  $250^\circ C$ , and while the gas flows and the internal pressure were stabilized, it was connected to the high frequency power source (739) and 200 watts power (frequency: 13.56 MHz) was applied to the power-applying electrode (736). After 35 plasma polymerization for approximately 4 hours, there was formed a charge transporting layer with a thickness of approximately 5 microns on the conductive substrate (752).

The ratio ( $N_3:N_4$ ) of  $N_3$  to  $N_4$  in the charge transporting layer was about 38:47.5, namely 1:1.25.

And then an a-Si charge generating layer was formed on the charge transporting layer obtained in the above process in a similar way as Example 8(II).

The photosensitive member thus obtained showed a half-reduced exposure value  $E_1$  of approximately 1.1 lux.sec for the initial surface potential ( $V_0$ ) = -500 volt. This photosensitive member, tested for the image transfer, produced clear images.

#### EXAMPLE 11

(I) In a system of glow discharge decomposition with equipment as illustrated in FIG. 13, first the reaction chamber (733) was vacuumized inside to a high level of approximately  $10^{-6}$  Torr, and then by opening No. 6 and No. 7 regulating valves (712) and (725),  $He$  gas from No. 6 tank (706) and styrene ( $C_8H_8$ ) gas from No. 1 vessel (719) were led into mass flow controller (718) and (728). No. 1 vessel (719) was heated at the temperature of about  $20^\circ C$  by No. 1 heater (722). Then, the mass flow controllers were set so as to make styrene flow at 40 sccm and  $He$  flow at 80 sccm, and the gases

were allowed into the reaction chamber (733). After the respective flows had stabilized, the internal pressure of the reaction chamber (733) was adjusted to 0.3 Torr. On the other hand, the electrically conductive substrate (752), which was an aluminum plate of  $2 \times 50 \times 50$  mm, was preliminarily heated up to 300° C., and while the gas flows and the internal pressure were stabilized, it was connected to the low frequency power source (741) and 150 watts power (frequency: 30 KHz) was applied to the power-applying electrode (736). After plasma polymerization for approximately 40 minutes, there was formed a charge transporting layer with a thickness of approximately 9 microns on the conductive substrate (752).

The ratio (N<sub>3</sub>:N<sub>4</sub>) of N<sub>3</sub> to N<sub>4</sub> in the charge transporting layer was 6:94, namely 1:15.7.

And then an a-Si charge generating layer was formed on the charge transporting layer obtained in the above process in a similar way as Example 8(II).

The photosensitive member thus obtained showed a half-reduced exposure value E<sub>1</sub> of 2.7 lux.sec for the initial surface potential (V<sub>0</sub>) = -560 volt. This photosensitive member had a practicable sensitivity, and tested for the image transfer, produced clear images.

#### EXAMPLE 12

Using the vapor deposition equipment of FIG. 14, titanylphthalocyanine was codeposited on an aluminum substrate under a vacuum of not more than  $1 \times 10^{-5}$  Torr, and the boat temperature of 400°-600° C., at the same time, ZnS was deposited under the boat temperature 900°-1150° C. The resultant codeposited layer had a thickness of 1000 Å.

Then, an a-C layer as a charge transporting layer was formed thereon with the same method as Example 5.

The ratio (N<sub>3</sub>:N<sub>4</sub>) of the above layer of the amount of unsaturated carbon N<sub>3</sub> linked with hydrogen to that of saturated carbon N<sub>4</sub> linked with hydrogen was 1:2.7.

The photosensitive member obtained above showed a half-reduced exposure value E<sub>1</sub> of 6.0 lux.sec for the initial surface potential (V<sub>0</sub>) of +550 volt.

Further, this member showed a half-reduced exposure value E<sub>1</sub> of 15.4 erg/cm<sup>2</sup> toward the semiconductor laser light having a wavelength of 780 nm.

Moreover, a photosensitive member was prepared to form the a-C layer of Example 6 on a charge generating layer made of non-crystal Se-Te or Se-As, each charge generating layer having a thickness of 1.2  $\mu$ m. The photosensitive members thus obtained showed excellent electrophotographic properties.

#### COMPARATIVE EXAMPLE 1

##### (I) Formation of an a-C Layer:

In a system of glow discharge decomposition with equipment as illustrated in FIG. 13, first the reaction chamber (733) was vacuumized inside to a high level of approximately  $10^{-6}$  Torr, and then by opening No. 1 and No. 2 regulating valves (707) and (708), H<sub>2</sub> gas from No. 1 tank (701), and pentane (C<sub>5</sub>H<sub>12</sub>) gas from No. 2 tank (702) were led, under output pressure gage reading of 1 Kg/cm<sup>2</sup>, into mass flow controllers (713) and (714). Then, the mass flow controllers were set so as to make H<sub>2</sub> gas flow at 300 sccm, and pentane gas flow at 100 sccm, and the gases were allowed into the reaction chamber (733). After the respective flows had stabilized, the internal pressure of the reaction chamber (733) was adjusted to 1.3 Torr. On the other hand, the electrically conductive substrate (752), which was an

aluminum plate of  $3 \times 50 \times 50$  mm, was preliminarily heated up to 260° C., and while the gas flows and the internal pressure were stabilized, it was connected to the high frequency power source (739) and 250 watts power (frequency: 13.56 MHz) was applied to the power-applying electrode (736). After plasma polymerization for approximately 8 hours, there was formed a charge transporting layer with a thickness of approximately 15 microns on the conductive substrate (752).

The ratio (N<sub>3</sub>:N<sub>4</sub>) of N<sub>3</sub> to N<sub>4</sub> in the charge transporting layer was 1:35, which was analyzed with the solid NMR system.

##### (II) Formation of a charge generating layer:

The power application from the high frequency power source (739) was stopped for a time and the reaction chamber was vacuumized inside.

By opening No. 1 and No. 6 regulating valves (707) and (712), H<sub>2</sub> gas from No. 1 tank (701) and SiH<sub>4</sub> gas from No. 6 tank (706) were, under output pressure gage reading of 1 Kg/cm<sup>2</sup>, led into the mass flow controllers (713) and (718). Then, the mass flow controllers were set so as to make SiH<sub>4</sub> flow at 100 sccm and H<sub>2</sub> flow at 200 sccm, and the gases were allowed into the reaction chamber. On the other hand, the electrically conductive substrate (752) with the a-C layer was preliminarily heated up to 250° C. After the respective flows had stabilized, the internal pressure of the reaction chamber (733) was adjusted to 0.8 Torr.

While the gas flows and the internal pressure were stabilized, the circuit to the high frequency power source (739) was supplied and a 35 W power (frequency: 13.56 MHz) was applied to the electrode (752) to generate glow discharge. After 5 minutes of glow discharge, there was formed an a-Si:H charge generating layer with a thickness of 0.3 micron.

The photosensitive member thus obtained was charged positively or negatively by means of the usual Carlson's process, and the results below were gained; Hereinafter the measured value when positively charged is given in parentheses. The highest charge voltage was -890 V (+895 V), but the amount of the white light necessary for reducing the surface voltage to the level of 20% of the highest charge voltage initially charged was 150 lux.sec (400 lux.sec).

It was understood that the sensitivity was too low for the photosensitive member obtained in the comparative example to be useful.

#### EXAMPLE 13

##### (I) Formation of an a-C layer:

In a system of glow discharge decomposition with equipment as illustrated in FIG. 13, first the reaction chamber (733) was vacuumized inside to a high level of approximately  $10^{-6}$  Torr, and then by opening No. 1 and No. 2 regulating valves (707) and (708), C<sub>2</sub>H<sub>4</sub> gas from No. 1 tank (701) and H<sub>2</sub> gas from No. 2 tank (702) were led, under output pressure gage reading of 1 Kg/cm<sup>2</sup>, into mass flow controllers (713) and (714). Then, the mass flow controllers were set so as to make C<sub>2</sub>H<sub>4</sub> flow at 30 sccm and H<sub>2</sub> flow at 65 sccm, and the gases were allowed into the reaction chamber (733). After the respective flows had stabilized, the internal pressure of the reaction chamber (733) was adjusted to 0.5 Torr. On the other hand, the electrically conductive substrate (752), which was an aluminum plate of  $2 \times 50 \times 50$  mm, was preliminarily heated up to 250° C.,

and while the gas flows and the internal pressure were stabilized, it was connected to the high frequency power source (739) and 100 watts power (frequency: 13.56 MHz) was applied to the power-applying electrode (736). After plasma polymerization for approximately four hours, there was formed a charge transporting layer with a thickness of approximately 6 microns on the conductive substrate (752).

The resultant plasma-polymerized ethylene layer is analyzed with the Fourier transform infrared absorption spectroscope (made by Perkin Elmer Ltd.), the  $^{13}\text{C}$ -NMR system (solid-NMR, made by Nippon Densi Ltd.) and  $^1\text{H}$ -NMR system (made by Nippon Densi Ltd.). In the chemical structure of the plasma-polymerized ethylene layer, the ratio (N<sub>5</sub>:N<sub>6</sub>) of the amount of unsaturated carbon N<sub>5</sub> free from linking with hydrogen and saturated carbon N<sub>6</sub> free from linking with hydrogen was approximately 1:4.56. The above layer had  $1.5 \times 10^{12} \Omega\text{-cm}$  or less of the dark specific resistance and  $10^2 - 10^4$  or more of the ratio of the dark specific resistance to the light specific resistance. The plasma-polymerized ethylene layer of the invention has been found to be applied effectively to a photosensitive member.

#### (II) Formation of a charge generating layer:

The power application from the high frequency power source (739) was stopped for a time and the reaction chamber was vacuumized inside.

By opening No. 3 and No. 2 regulating valves (709) and (708), SiH<sub>4</sub> gas from No. 3 tank (703) and H<sub>2</sub> gas from No. 2 tank (702) were, under output pressure gage reading of 1 Kg/cm<sup>2</sup>, led into the mass flow controllers (715) and (714). Then, the mass flow controllers were set so as to make SiH<sub>4</sub> flow at 90 sccm and H<sub>2</sub> flow at 210 sccm, and the gases were allowed into the reaction chamber. After the respective flows had stabilized, the internal pressure of the reaction chamber (733) was adjusted to 1.0 Torr.

While the gas flows and the internal pressure were stabilized, the circuit to the high frequency power source (739) was supplied and a 30 W power (frequency: 13.56 MHz) was applied to the power-applying electrode (736) to generate glow discharge. After 10 minutes of glow discharge, there was formed an a-Si:H charge generating layer with a thickness of 1 micron.

#### (III) Test of Property of photosensitive member:

The photosensitive member produced according to the above processes (I) and (II) was evaluated in its chargeability and sensitivity using the tester for a photosensitive member as illustrated in FIG. 15.

The sample of the photosensitive member produced (35) was put on the scanning table (37), and fixed by the shield cover (36). The scanning table (37) was moved to the charged area (52), and a high electric power supplied from the direct high electric power (40) of +7.7 KV was applied to the charger (42) to generate corona discharge on the surface of the photosensitive member, and then the scanning table (37) was moved to the discharge area (51). The surface potential of the corona discharged sample was sensed by the transparent electrode (48) to be indicated on the surface potential meter (49), and then put out on the recorder (50). The photosensitive member of the above showed an excellent chargeability.

Further, the shutter (47) was opened to irradiate the light from the halogen lamp (43), which was reflected

on the mirror (44), on the surface of the charged sample (35). The irradiation was effected through the transparent electrode (48), and the change of the surface potential by the irradiation was put out on the recorder (50) as well as the electric current at the same time was sensed by the photo-electric current monitor (38). The photosensitive member of the above showed a half-reduced exposure value E<sub>1/2</sub> of about 0.8 lux.sec for an initial surface potential (V<sub>0</sub>) of -490 volt.

Furthermore, a drum type of a photosensitive member was made in the same manner as the Example 1 excepting that the electric power of 250 W, the flow ratio of C<sub>2</sub>H<sub>2</sub> of 300 sccm, and the flow ratio of H<sub>2</sub> of 650 sccm were used as the condition of the production for the charge transporting layer, and the electric power of 250 W, SiH<sub>4</sub> of 80 sccm and H<sub>2</sub> of 500 sccm were used as the condition for the charge generating layer and assembled into the copying machine (EP-650Z) produced by Minolta Kamera K.k. to be tested for the image transfer. The obtained images were excellent.

A simulation test for a copying process was made using a tester of drum type photosensitive member (not shown). There was obtained a stable static electric property even after the repeat of 50000 times of full copying process (charge - exposure - transferring and charge for removal - erasing).

#### EXAMPLE 14

##### (I) Formation of an a-C Layer:

In a system of glow discharge decomposition with equipment as illustrated in FIG. 13, first the reaction chamber (733) was vacuumized inside to a high level of approximately  $10^{-6}$  Torr, and then by opening No. 1 and No. 2 regulating valves (707) and (708), C<sub>2</sub>H<sub>2</sub> gas from No. 1 tank (701) and H<sub>2</sub> gas from No. 2 tank (702) were led, under output pressure gage reading of 1 Kg/cm<sup>2</sup>, into mass flow controllers (713) and (714). Then, the mass flow controllers were set so as to make C<sub>2</sub>H<sub>2</sub> flow at 60 sccm and H<sub>2</sub> flow at 80 sccm, and the gases were allowed into the reaction chamber (733). After the respective flows had stabilized, the internal pressure of the reaction chamber (733) was adjusted to 0.8 Torr. On the other hand, the electrically conductive substrate (752), which was an aluminum plate of  $2 \times 50 \times 50$  mm, was preliminarily heated up to 200° C., and while the gas flows and the internal pressure were stabilized, it was connected to the high frequency power source (739) and 85 watts power (frequency: 13.56 MHz) was applied to the power-applying electrode (736). After plasma polymerization for approximately 1.2 hours, there was formed a charge transporting layer with a thickness of approximately 10 microns on the conductive substrate (752).

The ratio (N<sub>5</sub>:N<sub>6</sub>) of N<sub>5</sub> to N<sub>6</sub> in the charge transporting layer was about 40:60, namely 1:1.5.

##### (II) Formation of a charge generating layer:

The power application from the high frequency power source (739) was stopped for a time and the reaction chamber was vacuumized inside.

By opening No. 4 and No. 2 regulating valves (710) and (708), SiH<sub>4</sub> gas from No. 4 tank (704) and H<sub>2</sub> gas from No. 2 tank (702) were, under output pressure gage reading of 1 Kg/cm<sup>2</sup>, led into the mass flow controllers (716) and (714). Then, the mass flow controllers were set so as to make SiH<sub>4</sub> flow at 90 sccm and H<sub>2</sub> flow at

210 sccm, and the gases were allowed into the reaction chamber. After the respective flows had stabilized, the internal pressure of the reaction chamber (733) was adjusted to 1.0 Torr.

5 While the gas flows and the internal pressure were stabilized, the circuit to the high frequency power source (739) was supplied and a 30 W power (frequency: 13.56 MHz) was applied to the power-applying electrode (736) to generate glow discharge. After 10 minutes of glow discharge, there was formed an a-Si:H charge generating layer with a thickness of 1 micron.

10 The photosensitive member thus obtained showed a half-reduced exposure value  $E_{\frac{1}{2}}$  of 0.5 lux.sec for the initial surface potential ( $V_o$ ) = -460 volt. This photosensitive member, tested for the image transfer, produced clear images.

#### EXAMPLE 15

(I) In a system of glow discharge decomposition with equipment as illustrated in FIG. 13, first the reaction 20 chamber (733) was vacuumized inside to a high level of approximately  $10^{-6}$  Torr, and then by opening No. 1-No. 3 regulating valves (707)-(709),  $C_2H_4$  gas from No. 1 tank (701),  $CH_4$  gas from No. 2 tank (702) and  $H_2$  gas from No. 3 tank (703) were led, under output pressure gage reading of  $1\text{ Kg/cm}^2$ , into mass flow controllers (713)-(715). Then, the mass flow controllers were set so as to make  $C_2H_4$  flow at 45 sccm,  $CH_4$  flow at 100 sccm, and  $H_2$  flow at 120 sccm, and the gases were allowed into the reaction chamber (733). After the respective flows had stabilized, the internal pressure of the reaction chamber (733) was adjusted to 1.0 Torr. On the other hand, the electrically conductive substrate (752), which was an aluminum plate of  $2 \times 50 \times 50$  mm, was preliminarily heated up to  $250^\circ C$ , and while the 30 gas flows and the internal pressure were stabilized, it was connected to the high frequency power source (739) and 250 watts power (frequency: 13.56 MHz) was applied to the power-applying electrode (736). After plasma polymerization for approximately 6 hours, there was formed a charge transporting layer with a thickness of approximately 5.6 microns on the conductive substrate (752).

The ratio ( $N_5:N_6$ ) of  $N_5$  to  $N_6$  in the charge transporting layer was 10:90, namely 1:9.

45 And then, an a-Si charge generating layer was formed on the charge transporting layer obtained in the above process in a similar way as Example 14 (II).

The photosensitive member thus obtained showed a half-reduced exposure value  $E_{\frac{1}{2}}$  of 1.4 lux.sec for the 50 initial surface potential ( $V_o$ ) = -520 volt. This photosensitive member, tested for the image transfer, produced clear images.

#### EXAMPLE 16

(I) In a system of glow discharge decomposition with equipment as illustrated in FIG. 13, first the reaction chamber (733) was vacuumized inside to a high level of approximately  $10^{-6}$  Torr, and then by opening No. 1-No. 3 regulating valves (707)-(709),  $C_2H_4$  gas from No. 1 tank (701),  $CH_4$  gas from No. 2 tank (702) and  $H_2$  gas from No. 3 tank (703) were led, under output pressure gage reading of  $1\text{ Kg/cm}^2$ , into mass flow controllers (713)-(715). Then, the mass flow controllers were set so as to make  $C_2H_4$  flow at 55 sccm,  $CH_4$  flows at 60 sccm and  $H_2$  flow at 100 sccm, and the gases were allowed into the reaction chamber (733). After the respective flows had stabilized, the internal pressure of 65

the reaction chamber (733) was adjusted to 1.5 Torr. On the other hand, the electrically conductive substrate (752), which was an aluminum plate of  $2 \times 50 \times 50$  mm, was preliminarily heated up to  $250^\circ C$ , and while the gas flows and the internal pressure were stabilized, it was connected to the high frequency power source (739) and 200 watts power (frequency: 13.56 MHz) was applied to the power-applying electrode (736). After plasma polymerization for approximately 5 hours, there was formed a charge transporting layer with a thickness of approximately 5 microns on the conductive substrate (752).

The ratio ( $N_5:N_6$ ) of  $N_5$  to  $N_6$  in the charge transporting layer was about 44:56, namely 1:1.27.

15 And then, an a-Si charge generating layer was formed on the charge transporting layer obtained in the above process in a similar as Example 14 (II).

The photosensitive member thus obtained showed a half-reduced exposure value  $E_{\frac{1}{2}}$  of about 1.2 lux.sec for the initial surface potential ( $V_o$ ) = -500 volt. This photosensitive member, tested for the image transfer, produced clear images.

#### EXAMPLE 17

(I) In a system of glow discharge decomposition with equipment as illustrated in FIG. 13, first the reaction chamber (733) was vacuumized inside to a high level of approximately  $10^{-6}$  Torr, and then by opening No. 6 and No. 7 regulating valves (712) and (725), He gas from No. 6 tank (706) and styrene gas from No. 1 vessel (719) were led, under output pressure gage reading of  $1\text{ Kg/cm}^2$ , into mass flow controllers (718) and (728). The No. 1 vessel was heated at the temperature of about  $20^\circ C$  by No. 1 heater (722). Then, the mass flow controllers were set so as to make styrene ( $C_8H_8$ ) flow at 50 sccm and He flow at 30 sccm, and the gases were allowed into the reaction chamber (733). After the respective flows had stabilized, the internal pressure of the reaction chamber (733) was adjusted to 0.5 Torr. On the other hand, the electrically conductive substrate (752), which was an aluminum plate of  $3 \times 50 \times 50$  mm, was preliminarily heated up to  $150^\circ C$ , and while the gas flows and the internal pressure were stabilized, it was connected to the low frequency power source (741) and 40 150 watts power (frequency: 30 KHz) was applied to the power-applying electrode (736). After plasma polymerization for approximately 40 minutes, there was formed a charge transporting layer with a thickness of approximately 8 microns on the conductive substrate (752).

The ratio ( $N_5:N_6$ ) of  $N_5$  to  $N_6$  in the charge transporting layer was 63:37, namely 1:0.59.

45 And then, an a-Si charge generating layer was formed on the charge transporting layer obtained in the above process in a similar way as Example 14 (II).

The photosensitive member thus obtained showed a half-reduced exposure value  $E_{\frac{1}{2}}$  of 2.9 lux.sec for the initial surface potential ( $V_o$ ) = -650 volt. This photosensitive member had a practicable sensitivity, and tested for the image transfer, produced clear images.

#### COMPARATIVE EXAMPLE 2

##### (I) Formation of an a-C Layer:

65 In a system of glow discharge decomposition with equipment as illustrated in FIG. 13, first the reaction chamber (733) was vacuumized inside to a high level of approximately  $10^{-6}$  Torr, and then by opening No. 1

and No. 2 regulating valves (707) and (708), H<sub>2</sub> gas from No. 1 tank (701), and butane (C<sub>4</sub>H<sub>10</sub>) gas from No. 2 tank (702) were led, under output pressure gage reading of 1 Kg/cm<sup>2</sup>, into mass flow controllers (713) and (714). Then, the pass flow controllers were set so as to make H<sub>2</sub> flow at 240 sccm, and butane flow at 120 sccm, and the gases were allowed into the reaction chamber (733). After the respective flows had stabilized, the internal pressure of the reaction chamber (733) was adjusted to 1.5 Torr. On the other hand, the electrically conductive substrate (752), which was an aluminum plate of 3×50×50 mm, was preliminarily heated up to 270° C., and while the gas flows and the internal pressure were stabilized, it was connected to the high frequency power source (739) and 220 watts power (frequency: 13.56 MHz) was applied to the power-applying electrode (736). After plasma polymerization for approximately 15 hours, there was formed a charge transporting layer with a thickness of approximately 15 microns on the conductive substrate (752).

The ratio (N<sub>5</sub>:N<sub>6</sub>) of N<sub>5</sub> to N<sub>6</sub> in the charge transporting layer was 1:45.

#### (II) Formation of a charge generating layer:

The power application from the high frequency power source (739) was stopped for a time and the reaction chamber was vacuumized inside.

By opening No. 1 and No. 6 regulating valves (707) and (712), H<sub>2</sub> gas from No. 1 tank (701) and SiH<sub>4</sub> gas from No. 6 tank (706) were, under output pressure gage reading of 1 Kg/cm<sup>2</sup>, led into the mass flow controllers (713) and (718). Then, the mass flow controllers were set so as to make H<sub>2</sub> gas flow at 200 sccm and SiH<sub>4</sub> flow at 100 sccm, and the gases were allowed into the reaction chamber. On the other hand, the electrically conductive substrate (752) with the a-C layer was preliminarily heated up to 250° C. After the respective flows had stabilized, the internal pressure of the reaction chamber (733) was adjusted to 0.8 Torr.

While the gas flows and the internal pressure were stabilized, the circuit to the high frequency power source (739) was supplied and a 35 W power (frequency: 13.56 MHz) was applied to the electrode (752) to generate glow discharge. After 5 minutes of glow discharge, there was formed an a-Si:H charge generating layer with a thickness of 0.3 micron.

The photosensitive member thus obtained was charged positively or negatively by means of the usual Carlson's process, and the results below were gained; Hereinafter the measured value when positively charged is given in parentheses. The highest charge voltage was -920 V (+925 V), but the amount of the white light necessary for reducing the surface voltage to the level of 20% of the highest charge voltage initially charged was about 300 lux.sec (about 380 lux.sec).

It was understood that the sensitivity was too low for the photosensitive member obtained in the comparative example to be useful.

#### EXAMPLE 18

Using the vapor deposition equipment of FIG. 14, titanylphthalocyanine was codeposited on an aluminum substrate under a vaccum of not more than  $1 \times 10^{-5}$  Torr, and the boat temperature of 400°-600° C., at the same time, ZnS was deposited under the boat temperature 900°-1150° C. The resultant codeposited layer had a thickness of 1000 Å.

Then, an a-C layer as a charge transporting layer was formed thereon with the same method as Example 5.

The ratio (N<sub>5</sub>:N<sub>6</sub>) of the above layer of the amount of unsaturated carbon (N<sub>5</sub>) free from linking with hydrogen to that of saturated carbon (N<sub>6</sub>) free from linking with hydrogen was 1:2.0.

The photosensitive member obtained above showed a half-reduced exposure value E<sub>1/2</sub> of 6.0 lux.sec for the initial surface potential (V<sub>0</sub>) of +550 volt.

Further, this member showed a half-reduced exposure value E<sub>1/2</sub> of 15.4 erg/cm<sup>2</sup> toward the semiconductor laser light having a wavelength of 780 nm.

Moreover, a photosensitive member was prepared to form the a-C layer of Example 6 on a charge generating layer made of non-crystal Se-Te or Se-As, each charge generating layer having a thickness of 1.2 μm. The photosensitive members thus obtained showed excellent electrophotographic properties.

#### COMPARATIVE EXAMPLE 3

An a-Si:H layer with a thickness of 6 microns was formed in the identical process (II) with Example 1 (Process (I) for the production of a-C layer was cut out) to obtain an a-Si:H photosensitive member.

The photosensitive member thus obtained showed a half-reduced exposure value E<sub>1/2</sub> of 2.7 lux.sec for an initial surface potential (V<sub>0</sub>) = -100 V. The chargeability was inadequate when the polarity was positive, and the use of this photosensitive member failed to produce satisfactory images.

#### COMPARATIVE EXAMPLE 4

A plasma-polymerized polyethylene layer with the ratio (N<sub>1</sub>:N<sub>2</sub>) of N<sub>1</sub> to N<sub>2</sub> of more or equal to 1:1, the ratio (N<sub>3</sub>:N<sub>4</sub>) of N<sub>3</sub> to N<sub>4</sub> of less or equal to 1:1 or the ratio (N<sub>5</sub>:N<sub>6</sub>) of N<sub>5</sub> to N<sub>6</sub> of less or equal to 1:0.5 could not be formed even under various polymerizing condition. Although an a-C layer out of the range of the invention was once formed, it was soft and sticky and had not enough electric charge-transporting properties.

And that, a charge generating layer cannot be formed on the a-C layer because the a-C layer is deteriorated by temperature or plasma, so the a-C layer above cannot constitute a charge transporting layer of a photosensitive member.

#### COMPARATIVE EXAMPLE 5

Instead of the process (I) in Example 1 in the practice of the invention, a polyethylene layer with low density was formed as a charge transporting layer by a conventional method of an organic polymerization, and a charge generating layer was superimposed thereon by the process (II) in Example 1. The polyethylene layer had the ratio (N<sub>1</sub>:N<sub>2</sub>) of N<sub>1</sub> to N<sub>2</sub> of approximately  $1.5 \times 10^{-3}$ , and the ratio (N<sub>3</sub>:N<sub>4</sub>) of N<sub>3</sub> to N<sub>4</sub> of approximately 1:800. The ratio of the amount of carbon free from linking with hydrogen was 1% on the basis of all carbon in the polyethylene above, which was out of the range of 5-65%. The laminated layer obtained thereby

showed the specific electrical resistance of about  $10^{16}$  Ω.cm meaning insulator. The resultant photosensitive member was evaluated according to the process (III) in Example 1, but it had no photosensitivity and showed a charge-up phenomenon after a few repetitions. It cannot be used in reprography. This comparison attested the advantage of a charge transporting layer embodying the invention.

What is claimed is:

1. A photosensitive member comprising:  
an electrically conductive substrate;  
a charge generating layer; and  
a charge transporting layer comprising amorphous  
carbon containing hydrogen in an amount of 20 to  
67 atomic % and having a thickness of about 5 to  
about 50 microns, said amorphous carbon comprising  
hydrogen-bonded carbon N<sub>1</sub> and carbon N<sub>2</sub>  
free from linking with hydrogen, the ratio of the  
amount of N<sub>1</sub> to that of N<sub>2</sub> being 1:0.1 to 1:1, said  
hydrogen-bonded carbon N<sub>1</sub> comprising unsaturated  
carbon N<sub>3</sub> and saturated carbon N<sub>4</sub>, the ratio  
of the amount of N<sub>3</sub> to that of N<sub>4</sub> being about 1:1 to  
about 1:16, and said carbon N<sub>2</sub> free from linking  
with hydrogen comprising unsaturated carbon N<sub>5</sub>  
and saturated carbon N<sub>6</sub>, the ratio of the amount of  
N<sub>5</sub> to that of N<sub>6</sub> being about 1:0.5 to about 1:20.
2. A photosensitive member as claimed in claim 1  
wherein the ratio of the amount of N<sub>1</sub> to that of N<sub>2</sub> is  
preferably 1:0.2 to 1:0.8.
3. A photosensitive member as claimed in claim 1  
wherein the ratio of the amount of N<sub>3</sub> to that of N<sub>4</sub> is  
1:1.2 to 1:14.

25

30

4. A photosensitive member as claimed in claim 1  
wherein the amount of said carbon N<sub>2</sub> free from linking  
with hydrogen is 5 to 65% based on all carbon atoms.
5. A photosensitive member as claimed in claim 1  
wherein the ratio of the amount of N<sub>5</sub> to that of N<sub>6</sub> is 1:1  
to 1:10.
6. A photosensitive member comprising:  
an electrically conductive substrate;  
a charge generating layer; and  
a charge transporting layer comprising amorphous  
carbon containing hydrogen in an amount of 20 to  
67 atomic % and having a thickness of about 5 to  
about 50 microns, said amorphous carbon comprising  
hydrogen-bonded unsaturated carbon N<sub>3</sub> and  
hydrogen-bonded saturated carbon N<sub>4</sub>, the ratio of  
the amount of N<sub>3</sub> to that of N<sub>4</sub> being 1:1 to 1:16.
7. A photosensitive member comprising:  
an electrically conductive substrate;  
a charge generating layer; and  
a charge transporting layer comprising amorphous  
carbon containing hydrogen in an amount of 20 to  
67 atomic % and having a thickness of about 8 to  
about 80 microns, said amorphous carbon comprising  
unsaturated carbon N<sub>5</sub> free from linking with  
hydrogen and saturated carbon N<sub>6</sub> free from linking  
with hydrogen, the ratio of the amount of N<sub>5</sub> to  
that of N<sub>6</sub> being 1:0.5 to 1:20.

\* \* \* \* \*

35

40

45

50

55

60

65